

June 16, 1936.

C. E. YATES

2,044,415

METHOD AND APPARATUS FOR ELECTRODEPOSITION

Filed July 13, 1932

2 Sheets-Sheet 1

Fig. 2.



Fig. 1.



INVENTOR

Charles E. Yates  
By  
Pennie Days, Mawn, Edwards  
ATTORNEYS

June 16, 1936.

**C. E. YATES**

2,044,415

## METHOD AND APPARATUS FOR ELECTRODEPOSITION

Filed July 13, 1932

2 Sheets-Sheet 2

Fig. 3.



Fig. 4.



Fig. 5.



Fig. 6.



43



Fig. 7.



INVENTOR  
*Charles E. Gates*  
BY  
*Emmett Davis, Maxon, Edwards*  
ATTORNEYS

## UNITED STATES PATENT OFFICE

2,044,415

METHOD AND APPARATUS FOR  
ELECTRODEPOSITION

Charles E. Yates, Perth Amboy, N. J., assignor, by  
mesne assignments, to Anaconda Copper Min-  
ing Company, New York, N. Y., a corporation  
of Montana

Application July 13, 1932, Serial No. 622,171

35 Claims. (Cl. 204—6)

This invention relates to the electrolytic production of thin metallic sheets or foils by a procedure which involves plating metal on a cathode surface to the desired thickness and stripping it therefrom. More particularly, the invention is concerned with a novel method and apparatus by the use of which sheets and foils of either definite or indefinite dimensions can be produced, the deposited sheets having sharp clean-cut edges without increased thickness and the deposition being carried on under such conditions that plating of the metal on those surfaces of the cathode where it is not desired is prevented. The new method and apparatus may be used to especially advantage in the continuous production of thin copper foils and an embodiment of the invention in a form suitable for that purpose will accordingly be described in detail to make clear the principles involved, but it is to be understood that the utility of the invention is not limited to continuous production of foils of indefinite length nor to that particular metal.

The production of copper foils by plating on a rotating drum cathode and continuously stripping the deposit therefrom was proposed many years ago and numerous attempts have been made to develop such a process in a form which can be used commercially. These attempts, however, have heretofore not been successful because of numerous problems encountered, which up to the present have remained unsolved. One of the most important obstacles to commercial production of copper foils electrolytically is that of obtaining a product with sharp clean-cut edges and preventing deposition or sprouting on those surfaces of the drum where it is not desired.

To overcome the difficulty, it has been proposed, for example, to apply an insulating coating to the curved surface of the drum at its ends, to mount a strip of insulating material in the surface, or to apply a gasket or disc of insulating material to the ends of the drum, but while these expedients may function satisfactorily for a short time, they provide no permanent solution of the problem.

In the case of the insulated coating, the relatively high current density at the ends of the drum causes a powdery deposit of metal to occur along the edges of the insulated area. This deposit is not entirely removed by stripping, and the accumulated residue provides a good foundation for sprouts. In addition to sprouts thus formed, the electrolyte creeps under the edge of the coating and metal is deposited beneath 55 the coating. In the course of continued strip-

ping, this deposit is torn loose, destroying the coating. The formation of sprouts along the edge of the deposit surface results in the deposition of metal on an irregular edge surface, and when the sheet is stripped, serious troubles from 5 tearing of the sheet arise.

When gaskets at the ends of the drum or insulating material laid in a groove in the drum surface are used, sprouting occurs as before along the edge of the deposit surface, and in addition, 10 a thin layer of copper is deposited between the insulation and the drum, this layer remaining in place continuously. Tearing during stripping then arises from the presence both of the sprouts and the thin layer of copper under the insulation 15 and the latter is never removed during stripping and constitutes a continual cause of sprouting.

Another difficulty encountered in the use of a rotating drum apparatus in the continuous production of metal sheets is maintaining the surface of the drum in proper condition. In my co-pending application, Serial No. 604,932, filed April 13, 1932, I discussed this problem at some length and disclosed an apparatus by means of which the surface of the drum can be kept in 20 the desired condition for indefinite periods. That apparatus includes an element which abrades and smooths the surface of the drum after stripping and I have demonstrated that the particular apparatus disclosed is a solution of this problem. 30 It has been proposed by others working in this field to clean the surface of the drum by rotating brushes and various devices of that sort but all such devices, including my own, can be used only with some difficulty in connection with a 35 drum in which portions of the curved deposit surface are stopped off by insulating varnish or the like, since the operating element must be kept from contacting with the insulated area and at the same time all portions of the surface of 40 the cathode on which a deposit occurs must be treated.

The present invention is directed to a method and apparatus by which the difficulties in producing sheets with sharp well-defined edges are 45 overcome and sprouting on such surfaces of the drum as it is not desired to plate is prevented, the new apparatus being so constructed as to facilitate the necessary mechanical treatment of the curved surface of the drum to keep it in 50 proper condition.

In the deposition of metal on the surface of a drum cathode opposed by an anode, there is ordinarily a concentration of current along the end edges of the drum which results in the de- 55

posed sheet being built up to a greater thickness along its edges than elsewhere. Such increased current density on the cathode is caused by the face, edges, and back of the anode being exposed to the electrolyte, while the ends of the drum and in some cases portions of the curved surface of the drum at its ends are stopped off by an insulating coating. Accordingly, current entering the solution from the ends and back of the anode and seeking the nearest part of the cathode, flows to the cathode edges and this produces a current density along those edges which is higher than that on any other part of the cathode with a resultant deposition at a greater rate.

In one form of the apparatus embodying my invention, the drum may have circumferential channels in its curved surface adjacent the ends thereof and ports leading from the bottom of the channels and opening at the ends of the drum. The tops of the channels, at least throughout the length of those portions which lie beneath the electrolyte, are then covered by suitable means as, for example, rubber belts, and means are also employed for confining bodies of electrolyte in contact with those portions of the drum which are not to receive a plating. Such confining means may take the form of partition members mounted at the ends of the drum beyond the ends of the ports and extending from the drum to the tank wall. The electrolyte thus confined is kept separate from the main body of the electrolyte except for such slight leakage as may occur beneath the belts and partitions. In the confined bodies of electrolyte are placed cathodes, called "sub-cathodes" for convenience, which are maintained at a potential lower than that of the drum.

With this arrangement, the belts which cover the channels and also overlie the edge of the deposit surface along the channels to an extent dependent on the diameter of the belts, serve as a means for shielding the edges of the deposit surface and preventing increased thickness of the deposit along its edges. The belts alone may be sufficient to prevent increased thickness of the edges of the deposit but the action of the belts may be made more effective by providing non-conductive shields along the edges of the anode. If the belts and partition members made a perfect seal with the extreme edges of the deposit surface of the drum and with the tank wall, there would be no plating on any surface of the drum except that on which a deposit is desired. The belts and partition members, however, do not make such a seal and there is always some seepage of the electrolyte beneath the belts and between the partition members and the tank wall which would result in sprouting except for the presence of the sub-cathodes. Any stray currents which pass through the electrolyte leaking into the confined bodies at the ends of the drum flow at once to the sub-cathodes and by proper selection of voltages of the main cathode and the sub-cathodes, the latter may also cause a deplating of the deposit from the edges of the drum and thus assist the belts in preventing increased thickness at the edges of the deposit sheet. Ordinarily the belts with or without the anode shields are sufficient to control the thickness of the plating at the edges of the sheet and the sub-cathodes serve merely to prevent plating on those parts of the drum where no deposit is desired.

With the novel drum, therefore, the side edges

of the surface on which the foil is to be deposited are so defined and shielded that there can be no sprouting along these edges, and this result is obtained without the use of insulating coatings or the like on the surface of the cathode. The cathode surface may, therefore, be maintained in proper condition by the apparatus disclosed in my copending application above mentioned, and the use of the present apparatus with the surface treating mechanism disclosed in that application solves the problems of producing sheets of substantially uniform thickness with sharp clean edges and of maintaining the cathode surface in condition for continuous operation over long periods.

For a better understanding of the invention, reference may be had to the accompanying drawings illustrating one embodiment of the new apparatus. In these drawings,—

Fig. 1 is a vertical sectional view through the cell and drum cathode;

Fig. 2 is a view similar to Fig. 1 taken at right angles thereto;

Figs. 3 and 4 are sectional views through portions of the drum;

Fig. 5 is a diagrammatic view illustrating the electrical connections in a battery of cells; and

Figs. 6, 7 and 8 are diagrammatic views illustrating the flow of current between anodes and cathodes of various constructions.

Referring now to the drawings, the apparatus illustrated includes a tank 10 of any suitable material, the tank usually being lead lined, and mounted in bearings 11 at the top of the side walls of the tank is the shaft 12 of the drum 13. The drum has a surface which is to receive the deposit, this surface being the cylindrical surface of the drum and referred to as the "deposit surface". The remainder of the drum on which a deposit is not desired is referred to as the "non-deposit surface". The drum may be of any suitable construction but preferably includes spiders or discs 14 of copper constituting the ends of the drum and a cylindrical copper member 15 which provides the curved surface of the drum. The deposit surface is formed by a continuous layer 16 of lead mounted on the curved surface 15 and the ends of the drum are also provided with a lead sheathing so that the drum is completely enclosed and all its outer surfaces are covered with lead. The shaft of the drum is provided with a disc contact 17 which runs in a trough 18 containing mercury connected to the negative side of a source of energy.

In the bottom of the tank is a suitable support 19 for a pair of anodes 20, these anodes being of curved form and lying with their faces close to the cylindrical surface of the drum. The anodes are spaced apart at the bottom to provide a passage 21 and air agitation is used to maintain fresh electrolyte in the space between the anodes and cathode. For this purpose an air pipe 22 having jet openings at its top is mounted just below the passage, and the air promotes upward circulation of the electrolyte in the space between the anodes and the cathode. Each anode has lugs 23 which overlie and contact with bus bars 24 along the top of the tank, the bus bars being connected to a suitable source of current supply. The anodes are also preferably provided with shields 25 of insulating material along their lateral edges, these shields preventing current flow into the solution from the edges.

The lead plate 16 forming the outer cylindrical surface of the cathode projects beyond each end

of the drum a short distance, as illustrated in Fig. 3, and lead is filled in as at 16<sup>a</sup> to provide a flange extending beyond the end of the plate 16. The flange is then cut away to provide a circumferential channel 26 from the bottom of which ports 27 pass through the flange. A partition member 28 is mounted on the drum and extends therefrom to the wall of the cell, and I prefer to make this partition member of a pre-formed web of rubber and to secure it in place with a portion entering the channel 26. For this purpose, one side of the channel may be provided with a low circumferential rib 29 on flange 16<sup>a</sup> and the rubber web is placed in contact with the bottom of the channel and projects out over the top of the rib. After the rubber is drawn tightly in position and its ends secured together by rubber cement or the like, a clamping ring 30 of lead is placed to overlie a portion of the web and the ring is then drawn tightly together and its ends connected by burning to make it continuous. One side of the ring then forms one wall of the channel 26, and the ring is insulated from the drum.

25 That portion of each channel which lies below the level of the electrolyte is closed by means of an endless belt 31 of rubber which is trained about pulleys 32 mounted on the tank walls and has a portion free of the drum, this portion passing, for instance, across the end of the drum from one pulley to the other. The belts which I have found satisfactory have a rubber surface and are of circular section, the diameter being considerably greater than the width of the channel so that 35 the belts will overlie the edges of the deposit sheet and will make good contact with the top edges of the channel.

It will be observed that the belts 31 extend out beyond the drum a substantial distance, and, as 40 shown in Figs. 1 and 3, the size of the belts is such that they extend through a relatively large proportion of the distance between the drum and the anodes. The belts therefore reduce the openings at the ends of the drum into the space between the drum and anodes to a substantial extent, and since it is the current flowing through 45 these openings from the back of the anode and also from the end edges thereof (if these edges are unshielded) which produces the current concentration along the edges of the deposit surface and thickening of the edges of the sheet, it will 50 be apparent that by reducing the size of the openings between the anode and drum adjacent the ends of the drum, the belts reduce the current flow referred to and, consequently, prevent 55 thickening of the sheet along its edges. In order that they may be used satisfactorily for this purpose, the belts must extend out beyond the cathode to a substantial extent and must provide 60 a substantial restriction of the path of current flow. If the belts do not extend out beyond the cathode in the manner described, or the anodes are so spaced from the cathode that there is no substantial restriction of current flow by the belts, 65 edge thickening of the sheet will not be prevented or reduced by the belts.

One or more sub-cathodes 34 are mounted at the ends of the drum and they may be secured to insulating bases 35 secured to the tank walls, the sub-cathodes at each end of the drum being immersed in a body of electrolyte which is confined within the circular partition at that end of the drum. In the construction illustrated in Figs. 1 and 2, there are two sub-cathodes at each end of the drum. These sub-cathodes are main-

tained at a potential lower than that of the main cathode and this may be done by properly connecting the sub-cathodes in the electrical system to which the main cathode is connected or by providing a separate system for the sub-cathodes. 5 Instead of mounting the sub-cathodes on the tank wall, a ring of conducting material may be mounted on an insulating base 37 on each end of the drum, the contact being made with the ring by suitable brushes. 10

A battery of tanks is illustrated in Fig. 5, and these tanks are advantageously connected in series, with the anodes 38 of the first tank in the series connected to the positive side of the source of energy. The main cathode in the first tank 15 is then connected through a line 39 to the anodes 40 in the second tank and the main cathode 41 in the second tank is connected by a line 42 to the anodes 43 in the third tank. The sub-cathodes in any tank can then be connected to any point 20 in the system beyond the main cathode in the next later tank in the series. In the lay-out illustrated, a branch connection 44 from the line 42 leads back to the sub-cathodes 45 in the first tank, the sub-cathodes thus being maintained at 25 a potential less than the main cathode in that tank. Similar connections are provided throughout the battery of the tanks so that current is supplied to the tanks in series and the sub-cathodes in each tank have a lower potential than the 30 main cathode in that tank. The sub-cathodes in the last tank in the series are then maintained at their proper potentials either by being connected electrically to some point in the tank house 35 at the proper potential or separate means for maintaining those sub-cathodes at the proper potential may be employed.

The use of the sub-cathodes with a cathode drum of the construction described prevents 40 sprouting on the end surfaces of the drum and the formation of a deposit along the edges of the drum surface, which eventually produces ragged edges on the sheet. The sub-cathodes may also assist in preventing the deposit from becoming 45 thickened along its edges. I am aware that in electroplating operations, it has been proposed to use a secondary cathode known as a "thief" to prevent plating on surfaces where such plating is not desired, but in the apparatus with which I am familiar, the thief is connected to the main 50 cathode so that the two have the same potential. The purpose of such a thief is to divide the current flow, a portion of the metal leaving the solution being deposited on the main cathode and another portion on the thief. The action of the thief is then controlled by making it of proper 55 shape and size and by varying its position relative to the main cathode.

The function of a thief is quite different from that of my sub-cathode and the action of the latter is controlled in a different way. The sub-cathode is maintained at a potential lower than that of the main cathode so that the latter has the relation of an anode to the sub-cathode, and the action of the sub-cathode is controlled by 65 varying the difference in potential between the main cathode and the sub-cathode. The confined body of electrolyte in which the sub-cathode is immersed is in contact with those surfaces of the main cathode which are not to receive a deposit, 70 and is substantially isolated from the main body of the electrolyte except for such leakage as may take place between the edges of the channels and the belts and between the partitions and the tank wall. In the electroplating apparatus of the gen- 75

eral type disclosed, it is customary to employ a voltage drop of  $2\frac{1}{2}$  volts between the anode and main cathode in each cell and with the electrical connections as illustrated in Fig. 5, there would be a voltage drop of  $2\frac{1}{2}$  volts between the main cathode and the sub-cathode in each cell assuming there is no resistance in the connections. The drop between the main cathode and the sub-cathode, however, can be controlled by the introduction of resistance in the connections and will usually be of the order of half a volt. With that arrangement, substantially all current entering a confined body of electrolyte through a leakage path flows to the sub-cathode and causes a deposit thereon. If any metal is deposited from the confined body of electrolyte on the end of the drum, it can be easily removed by increasing the voltage drop from the drum to the sub-cathode but ordinarily a drop of  $\frac{1}{2}$  volt serves the desired purpose.

The drum illustrated in Fig. 3 has the advantage that its surface may be maintained in proper condition by the treating mechanism disclosed in my copending application above-identified. The lead clamping ring 30 which holds the rubber partition in place in the Fig. 3 construction will have its outer surface either flush with the cylindrical surface of the cathode or slightly lower and an operating element of a size sufficient to insure proper treatment of all portions of the surface of the drum may then be used, since the contact of the element with the ring causes no trouble and if the surface of the ring lies flush with the surface of the drum at the beginning of operations, the two will be worn down equally by the treating mechanism. This construction, however, necessitates the application of the clamping rings at the ends of the drum, and the somewhat simpler drum construction illustrated in Fig. 4 may be used in processes in which stripping is effected by the use of a stripping agent and the surface of the drum is not acted on by mechanical means which would wear it down.

In the Fig. 4 construction, the drum is formed with a circumferential channel 46 near each end and a rubber partition member 47 of L-section is then mounted so that one leg of the L enters the channel. The partition member is held in place in any suitable way and it projects out beyond the end of the drum so as to contact with the cell wall. With this construction, the rubber belt 31 contacts directly with the partition member at one side of the channel.

In Figs. 6, 7 and 8, the current conditions at the ends of a cathode drum are diagrammatically illustrated and in Fig. 6 there is shown an anode 48 opposing the face of a cathode 49, the end of which is stopped off by means of insulating material. The light lines extending from the anode to the cathode represent the flow of current and it will be apparent that along the edge of the cathode, there is a relatively high current density because of current entering the electrolyte from the edge and back of the anode.

In Fig. 7 current flows from the face and edge of anode 48 to the face of cathode 50, which is of my new construction. The presence of the belt 31 now presents a considerable obstruction to current flow and less current enters the solution from the end of the anode because of the difficulty of reaching the cathode, and most of the current passes directly from the face of the anode to the face of the cathode. At the same time, a small amount of current may flow through electrolyte

which seeps beneath the belt and through the confined body of electrolyte to the sub-cathode.

In Fig. 8, the cathode 50 is of the new construction and the anode is provided with an insulating shield 25 along its edge which prevents current entering the solution from that edge. In this case an increase of current density along the edge of the cathode is prevented both by the belt 31 and the shield 25.

I have found that with the new method and apparatus, sheets and foils of indefinite length may be produced as a commercial operation continuing for indefinite periods. The material produced is of substantially uniform thickness from edge to edge and the edges are sharp and well defined. Also, since sprouting at the edges of the deposit surface is prevented, difficulties in stripping, which have heretofore resulted in tearing the deposited sheet, are wholly prevented.

What I claim is:

1. A method of electrodeposition carried on in a cell containing an electrolyte, an anode, a cylindrical main cathode having its curved surface opposed to the anode, and a sub-cathode opposed to the end of the main cathode which comprises causing current to flow through the electrolyte from the anode to the curved surface of the cathode, confining a body of electrolyte in contact with the end of the main cathode and the sub-cathode, said body of electrolyte being isolated from the remainder of the electrolyte maintaining said sub-cathode at a potential lower than that of the main cathode, and maintaining a continuous circulation of electrolyte through the space between the main cathode and the anode.

2. Apparatus for electrodeposition comprising an electrolytic cell containing an electrolyte, an anode in the cell, a main cathode in the cell having a deposit surface and a non-deposit surface, said deposit surface being opposed to the surface of the anode, a sub-cathode in the cell having its surface opposed to said non-deposit surface, means for confining a portion of the electrolyte in contact with the sub-cathode and said non-deposit surface of the main cathode and isolating said portion of the electrolyte from the remainder, and means for maintaining the sub-cathode at a lower potential than that of the main cathode.

3. Apparatus for electrodeposition which comprises an electrolytic cell containing an electrolyte, an anode in the cell, a main cathode in the cell, said cathode being of cylindrical drum form with its curved surface opposed to the anode, a sub-cathode in the cell opposed to an end of the drum, means for confining a body of electrolyte in contact with the main cathode and the sub-cathode and isolated from the remainder of the electrolyte, and means for maintaining the sub-cathode at a potential lower than that of the main cathode.

4. Apparatus for electrodeposition which comprises an electrolytic cell containing an electrolyte, an anode in the cell, a main cathode in the cell, said cathode being of cylindrical drum form with its curved surface opposed to the anode, a sub-cathode in the cell opposed to an end of the drum, means for maintaining the sub-cathode at a potential lower than that of the main cathode, means for confining a body of the electrolyte in contact with the main cathode and the sub-cathode and isolated from the remainder of the electrolyte, and means for causing a circulation of the remainder of the electrolyte between the opposed surfaces of the main cathode and the anode.

5. Apparatus for electrodeposition which comprises an electrolytic cell containing an electrolyte, an anode in the cell, a main cathode in the cell, said cathode being of cylindrical drum form with its curved surface opposed to the anode, a sub-cathode mounted on the wall of the cell in opposition to an end of the main cathode, means for confining a portion of the electrolyte in contact with the end of the main cathode and with the sub-cathode and isolated from the remainder of the electrolyte and means for maintaining the sub-cathode at a potential lower than that of the main cathode.
10. Apparatus for electrodeposition which comprises an electrolytic cell containing an electrolyte, an anode in the cell, a main cathode in the cell, said cathode being of cylindrical drum form with its curved surface opposed to the anode, a sub-cathode mounted on the end of the main cathode and insulated therefrom, means for confining a body of electrolyte in contact with the end of the main cathode and the sub-cathode and isolated from the remainder of the electrolyte and means for maintaining the sub-cathode at a potential lower than that of the main cathode.
15. Apparatus for electrodeposition which comprises an electrolytic cell containing an electrolyte, an anode in the cell, a cylindrical drum main cathode in the cell having its curved surface opposed to the anode to receive a deposit, a sub-cathode in the cell opposed to the end of the drum, means extending between the end of the drum and the wall of the cell for confining a body of electrolyte in contact with the end of the drum and the sub-cathode and isolated from the remainder of the electrolyte, and means for maintaining the sub-cathode at a potential lower than that of the main cathode.
20. Apparatus for electrodeposition which comprises an electrolytic cell containing an electrolyte, an anode in the cell, a cylindrical drum main cathode in the cell having its curved surface opposed to the anode to receive a deposit, a sub-cathode in the cell opposed to the end of the drum, means carried by the drum and contacting with the wall of the cell for confining a body of electrolyte in contact with the end of the drum and the sub-cathode and isolated from the remainder of the electrolyte, and means for maintaining the sub-cathode at a potential lower than that of the main cathode.
25. Apparatus for electrodeposition which comprises an electrolytic cell containing an electrolyte, a cylindrical drum main cathode in the cell, an anode in the cell said anode being curved and mounted to oppose the curved surface of the drum, a sub-cathode in the cell opposing an end of the drum, means for confining a body of electrolyte in contact with the end of the drum and the sub-cathode, means for maintaining the sub-cathode at a potential lower than that of the main cathode.
30. Apparatus for electrodeposition which comprises an electrolytic cell containing an electrolyte, a cylindrical drum main cathode in the cell, an anode in the cell said anode being curved and mounted to oppose the curved surface of the drum, a sub-cathode in the cell opposing an end of the drum, means for causing a continuous flow of electrolyte in the space between the main cathode and the anode.
35. Apparatus for electrodeposition which comprises an electrolytic cell containing an electrolyte, a cylindrical drum cathode mounted to have a portion of its curved surface immersed in the electrolyte in said cell, a circumferential channel formed in the curved surface of the drum near each end thereof, ports extending through said surface from the bottom of each channel, and an endless belt covering the top of each channel throughout at least a portion of the circumference of the drum.
40. Apparatus for electrodeposition which comprises an electrolytic cell containing an electrolyte, a cylindrical drum cathode mounted to have a portion of its curved surface immersed in the electrolyte in said cell, a circumferential channel formed in the curved surface of the drum near each end thereof, ports extending through said surface from the bottom of each channel, pairs of rotary guides, a pair near each end of the drum and above the level of the electrolyte in the cell, and a pair of belts, one at each end of the drum, each belt passing around one pair of guides and having a portion covering the top of that portion of the channel which lies beneath the electrolyte.
45. Apparatus for electrodeposition which comprises an electrolytic cell containing an electrolyte, a cylindrical drum cathode mounted to have a portion of its curved surface immersed in the electrolyte in the cell, and an open circumferential channel in the curved surface of the drum near at least one end thereof.
50. Apparatus for electrodeposition which comprises an electrolytic cell containing an electrolyte, a cylindrical drum cathode mounted to have a portion of its curved surface immersed in the electrolyte in the cell, a circumferential channel near at least one end thereof, and ports leading through the curved surface from said channel.
55. Apparatus for electrodeposition which comprises an electrolytic cell containing an electrolyte, a cylindrical drum cathode mounted to have a portion of its curved surface immersed in the electrolyte in the cell, a circumferential channel near at least one end thereof, and a non-conductive partition member mounted at at least one end of the drum and extending through the curved surface from said channel.
60. Apparatus for electrodeposition which comprises an electrolytic cell containing an electrolyte, a cylindrical drum cathode mounted to have a portion of its curved surface immersed in the electrolyte in the cell, a circumferential channel near at least one end thereof, and a flexible web mounted at at least one end of the drum and extending edgewise toward and engaging the wall of the cell.
65. Apparatus for electrodeposition which comprises an electrolytic cell containing an electrolyte, a cylindrical drum cathode mounted to have a portion of its curved surface immersed in the electrolyte in the cell, a circumferential channel near at least one end thereof, and a rubber web attached to the drum and extending edgewise toward and engaging the wall of the cell, said web confining a body of electrolyte between the end of the drum and said wall.
70. Apparatus for electrodeposition which comprises an electrolytic cell containing an electrolyte, a cylindrical drum cathode mounted to have a portion of its curved surface immersed in the electrolyte in the cell, a circumferential channel near at least one end thereof, and a partition member mounted at at least one end of the drum and extending from one side of the channel to the wall of the cell.
75. Apparatus for electrodeposition which comprises an electrolytic cell containing an electrolyte, a cylindrical drum cathode mounted to have a portion of its curved surface immersed in the electrolyte in the cell, a circumferential channel in the curved surface of the drum at at least one end thereof, a cylindrical partition member projecting beyond said end of the drum and engaging the wall of the cell, and a ring holding said member in place.

20. In an electrolytic cell, the combination of a cylindrical drum cathode mounted to have a portion of its curved surface immersed in the electrolyte in the cell, a circumferential channel in the curved surface of the drum at at least one end thereof, a cylindrical partition member projecting beyond said end of the drum and engaging the wall of the cell, and a ring overlying said member to hold it in place, said ring defining a part of said channel.
21. In an electrolytic cell, the combination of a cylindrical drum cathode mounted to have a portion of its curved surface immersed in the electrolyte in the cell, and a partition member mounted on the drum and extending toward the wall of the cell.
22. Apparatus for electrodeposition which comprises a tank containing an electrolyte, an anode in the tank, a cathode in the tank having a surface opposing and spaced from the anode for receiving a deposit and another surface exposed to the electrolyte but on which no deposit is desired, means for supplying current to the anode and withdrawing it from the cathode, mechanical means adjacent the edges of the deposit surface of the cathode for preventing thickening of the plating along said edges, said means substantially restricting access of electrolyte to the space between the anode and cathode, and electrical means for preventing deposition on the surface of the cathode on which no deposit is desired.
23. Apparatus for electrodeposition comprising a tank containing an electrolyte, a rotating drum cathode having a portion of its cylindrical surface continuously immersed in the electrolyte, an anode in the tank opposing the curved surface of the drum and spaced therefrom, means for supplying current to the anode and withdrawing it from the cathode, mechanical means adjacent the ends of the drum for preventing thickening of the deposit on the curved surface of the drum, said means substantially restricting access of electrolyte to the flow of current through the openings at the ends of the drum cathode into the space between the anode and said curved surface, and electrical means for preventing deposition on the ends of the drum.
24. Apparatus for electrodeposition comprising a tank containing an electrolyte, a rotating drum cathode having a portion of its cylindrical surface continuously immersed in the electrolyte, an anode in the tank opposing the curved surface of the drum and spaced therefrom, means for supplying current to the anode and withdrawing it from the cathode, members mounted on the curved surface of the drum adjacent the ends thereof and extending from said surface toward the anode a substantial distance so as to reduce the size of the openings at the ends of said cylindrical surface into the space between the anode and said surface to a substantial extent, and electrical means for preventing deposition on the ends of the drum.
25. A method of electrodeposition carried on in a cell containing electrolyte, an anode, a main cathode having a deposit and a non-deposit surface, and a sub-cathode, which comprises maintaining a main body of electrolyte in contact with the anode and with the deposit surface of the main cathode, maintaining said sub-cathode at a potential lower than that of the main cathode and out of contact with said main body of electrolyte and immersed in a second body of electrolyte substantially isolated from said main body, said second body being in contact with the non-deposit surface of the main cathode, introducing current into the cell through the anode, and withdrawing current from the cell simultaneously through the main cathode and through the sub-cathode.
26. A method of electrodeposition carried on in a group of cells, each containing electrolyte, an anode, a main cathode having a deposit and a non-deposit surface, and a sub-cathode, which comprises maintaining in each cell a body of electrolyte in contact with the anode and with the deposit surface of the main cathode, maintaining in each cell a body of electrolyte substantially isolated from the first-mentioned body of electrolyte in said cell and in contact with the sub-cathode and with the non-deposit surface of the main cathode, introducing current into the electrolyte in each cell in the series through the anode in said cell, withdrawing current from each cell simultaneously through the main cathode and the sub-cathode in said cell, delivering the current withdrawn through the main cathode of each cell except the last to the anode of the next succeeding cell in the series, and delivering the current withdrawn from each cell except the last cell through the sub-cathode in said cell to the cathode of said next succeeding cell in the series.
27. Apparatus for electrodeposition which comprises a plurality of electrolytic cells, each containing electrolyte, an anode, a main cathode having a deposit and a non-deposit surface, and a sub-cathode, means in each cell for confining a body of electrolyte therein in contact with the sub-cathode and with the non-deposit surface of the main cathode, said body of electrolyte being substantially isolated from the remainder of the electrolyte which is in contact with the anode and the deposit surface of the main cathode, means for supplying current from the positive side of a source of energy to the anode of the first cell in the series, means for withdrawing current from the main cathode of the last cell in the series and delivering it to the negative side of the source of energy, connections outside the cells between the main cathode of each cell except the last and the anode of the next succeeding cell in the series, and means for maintaining the sub-cathode in each cell at a potential lower than the main cathode in its cell, said means serving to withdraw current from each cell through its sub-cathode.
28. A method of electrodeposition carried on in a cell containing electrolyte, an anode, a main cathode having a deposit and a non-deposit surface, and a sub-cathode, which comprises maintaining a main body of electrolyte in contact with the anode and the deposit surface of the main cathode, maintaining a body of electrolyte substantially isolated from the body first mentioned and in contact with the sub-cathode and with the non-deposit surface of the main cathode, said sub-cathode being out of contact with said main body of electrolyte, introducing current into the cell through the anode, withdrawing current from the cell simultaneously through the main cathode and the sub-cathode, and varying the relative proportions of the current withdrawn from the cell through the main cathode and the sub-cathode by varying the voltage drop between the main cathode and the sub-cathode, through the substantially isolated body of electrolyte.
29. A method of electrodeposition carried on

in a cell containing electrolyte, an anode, a main cathode having a deposit and a non-deposit surface, and a sub-cathode, which comprises maintaining a main body of electrolyte in contact with 5 the anode and the deposit surface of the main cathode, maintaining a body of electrolyte substantially isolated from the body first-mentioned and in contact with the sub-cathode and with the non-deposit surface of the main cathode, said 10 sub-cathode being out of contact with said main body of electrolyte introducing current into the cell through the anode, withdrawing current from the cell simultaneously through the main cathode and the sub-cathode, and shielding the lateral edges of the deposit surface on the main cathode to prevent increased current density 15 thereon.

30. Apparatus for electrodeposition comprising a tank containing an electrolyte, an anode 20 in the tank, a cathode in the tank having a deposit surface and a non-deposit surface both exposed to the electrolyte, means for confining a portion of the electrolyte in contact with the non-deposit surface of the cathode and substantially isolated from the remainder of the electrolyte which is in contact with the anode and the deposit surface of the cathode, means for supplying current to the anode, mechanical means for preventing thickening of the plating 25 30 along the edges of the deposit surface of the main cathode, and electrical means for preventing deposition on the non-deposit surface of the cathode, said electrical means also withdrawing current from the confined body of electrolyte only.

31. Apparatus for electrodeposition comprising a tank containing an electrolyte, a rotating drum cathode, this cathode having a deposit surface and a non-deposit surface, both of which 40 have portions continuously immersed in the electrolyte, means for confining a body of electrolyte in contact with the non-deposit surface of the cathode and substantially isolated from the remainder of the electrolyte which is in contact with the deposit surface of the cathode, an anode in the tank, means for supplying current to the anode and withdrawing it from the cathode, mechanical means for preventing thickening of the plating along the edges of the deposit 45 50 surface of the cathode, and electrical means for preventing deposition on the non-deposit surface of the cathode, said means also serving to withdraw current from the confined body of the electrolyte only.

55. 32. A method of electrodeposition carried on in a tank containing electrolyte, an anode, a main cathode having a deposit surface and a non-deposit surface, and a sub-cathode, which comprises circulating electrolyte in contact with 60 the deposit surface of the main cathode and with the anode, maintaining a portion of the electrolyte substantially stagnant and isolated

from the remainder of the electrolyte, said isolated electrolyte being in contact with the sub-cathode and the non-deposit surface of the main cathode, maintaining the sub-cathode out of contact with said circulating electrolyte and at a potential lower than that of the main cathode, introducing current into the tank through the anode, and withdrawing current from the tank simultaneously through the main cathode and the sub-cathode. 10

33. Apparatus for electrodeposition which comprises a tank containing electrolyte, an anode in the tank, a main cathode in the tank having a deposit surface and a non-deposit surface, means for circulating the electrolyte in contact 15 with the anode and the deposit surface of the cathode, means for confining and keeping out of circulation a portion of the electrolyte in contact with the non-deposit surface of the main cathode, a sub-cathode in contact with said portion of the electrolyte and out of contact with the circulating electrolyte, means for introducing current into the tank through the anode, and means for withdrawing current from the tank simultaneously through the main cathode 20 and through the sub-cathode. 25

34. In a metal plating operation, the method of controlling the deposition of metal on a selected area of an object which comprises, immersing the object in an electrolyte in a cell 30 containing an anode, attaching the object as a cathode to a source of current to effect deposition of metal upon a part of the surface of said object, isolating from the main body of electrolyte that portion of the electrolyte which contacts with another area on said object upon which the deposition is to be controlled, immersing an electrically conducting member in said isolated portion of the electrolyte, said member being out of electrical contact with said object, 40 and maintaining said member at a potential lower than that of the object. 45

35. Apparatus for electrodeposition which comprises, a tank containing an electrolyte, an anode in the tank, a cathode in the tank having a surface upon which metal is to be deposited and a second surface upon which the deposition is to be controlled, means for supplying current to the anode and withdrawing it from the cathode, means for isolating from the 50 main body of electrolyte a portion of the electrolyte which contacts with said second surface, the deposition on which is to be controlled, an electrically conducting member in said isolated portion of electrolyte, said member being out of 55 electrical contact with said cathode, and means for maintaining said member at a potential sufficiently lower than that of said cathode to control the deposition on said surface of the cathode. 60

CHARLES E. YATES.